

July 25, 1950

W. A. HARE ET AL

2,516,316

BORAX SPINNING BATH

Filed July 14, 1949



INVENTORS:  
WESTON ANDREW HARE  
FRANK KERR SIGNAIGO  
BY

*C. H. Montessori*  
ATTORNEY

## UNITED STATES PATENT OFFICE

2,516,316

## BORAX SPINNING BATH

Weston Andrew Hare, Kenmore, N. Y., and Frank Kerr Signaigo, Wilmington, Del., assignors to E. I. du Pont de Nemours & Company, Wilmington, Del., a corporation of Delaware

Application July 14, 1949, Serial No. 104,613

17 Claims. (Cl. 18—54)

2

This invention relates to the manufacture of regenerated cellulose articles and it is particularly concerned with improvements in the art of making high tenacity rayon from viscose.

Various methods have heretofore been suggested for making rayon from viscose and a number of these processes have involved the stretching of the filaments for the purpose of improving tenacity and otherwise modifying the physical characteristics of the filaments. These previously known processes are subject however to certain limitations, particularly with respect to the degree of stretch which can be imparted to the filaments and also with respect to the inability to produce very high tenacity yarn having the proper physical characteristics. This narrows the field of the utility of the processes and products. It has been found in accordance with the present invention that defects encountered in previous practice can be overcome by the use of novel spinning baths and carefully controlled conditions of filament formation and treatment.

It is an object of this invention to provide a new and improved process for the manufacture of regenerated cellulose articles. A further object comprehends the production of rayon having improved physical characteristics. An additional object pertains to the use of a special type of coagulating bath in forming regenerated cellulose products. Another object relates to the production of cellulose xanthate filaments which can be stretched to a considerable degree and which, upon regeneration, yield a product having a very high tenacity. Other objects of the invention will become apparent hereinafter.

The objects of the invention are accomplished in general by extruding viscose into a bath containing dissolved therein a substantial amount of a borate, being an amount equivalent to at least 5% of borax and maintained under such conditions as to precipitate the cellulose xanthate rapidly without substantially converting it to regenerated cellulose. Thereafter the water-soluble cellulose xanthate structure is preferably stretched a very substantial amount and then converted to regenerated cellulose by the use of any suitable treatment following which the product is washed, purified and dried.

One form of apparatus, suitable for use in carrying out the process of the present invention is illustrated in the accompanying drawing.

Figure 1 is a diagrammatic, side elevational view, with parts shown in section, of an apparatus particularly desirable for operation in accordance with the description set forth in Example I, below.

Referring to the drawing, a viscose filament-forming composition is forced through candle-filter 2, "gooseneck" 3, and spinnerette 4 in the conventional manner. The filaments 6 issue from spinnerette 4 below the surface of the spinning bath in tank 5. From the spinnerette the filaments 6 are passed about feed wheel 7 and cooperating guide roller 8, then about rollers 10 and 11 positioned in the stretching bath in tank 9, then about feed wheel 12 and cooperating guide roller 13. The yarn is passed about the two feed wheels 7 and 12 with a sufficient number of turns to prevent slippage of the yarn. Feed wheel 12 is rotated at a higher speed than feed wheel 7 so as to impart a stretch to the filaments passing through the bath in tank 9.

From feed wheel 12, the yarn drops of its own weight onto eccentrically revolving plate 14 to build up the yarn cake 15. The eccentrically revolving plate is of the type described in U. S. Patent to Dannenberg et al. No. 2,089,159.

For convenience, the invention will be described with particular reference to rayon although in its broader aspects it is applicable to the manufacture of articles having a physical shape or form different from rayon.

The following examples describe various modes of practicing the invention and in these examples, which are intended to illustrate rather than restrict the invention, parts and proportions are by weight unless otherwise specified.

## Example I

Viscose containing 5% cellulose and 9% sodium hydroxide and having a common salt (sodium chloride) index of 2.0 was extruded through a spinnerette into a bath prepared from 20% borax ( $Na_2B_4O_7 \cdot 10H_2O$ ), 10% sodium sulfate and 70% water, to which is added sufficient sulfuric acid to yield a pH of 4.0. The bath was maintained at approximately 60° C. The filaments were passed through the bath for a distance of 6 inches without contact with guides or any other device which may impart tension and were then withdrawn from the bath and passed through air at normal room conditions (75° F. and atmospheric pressure) for a distance of 8 inches to a positively driven glass roller or feed wheel which imparts to the filaments a speed of 300 inches per minute. The filaments are passed around the glass draw-off roller five times to prevent slippage using grooved rollers freely mounted to keep the yarn passes separated, which travel therearound was equal to about 130 inches. The filament were passed for a distance of 20

inches through a second bath around two submerged grooved rollers and thence to the second stretch roller or feed wheel positively driven to impart a speed to the filaments of 1020 inches per minute. The stretching bath composition was 10% borax, 10% sodium sulfate and 80% water, with the addition of sufficient sulfuric acid to yield a pH of 5.6. Under these conditions the filaments become stretched through the second bath to 3.4 times their original length, i. e. 10 their length at the first driven roller (the stretch thus being 240%). This second bath was maintained at boiling temperature. The yarn leaving the second positively driven roller was allowed to fall of its own weight on to a flat plate which is so moved as to traverse the yarn according to any desired pattern and thus build up a suitable cake or package. The filaments of yarn at this point were still in the form of cellulose xanthate free from any substantial degree of regeneration. The cake was then covered with a cloth wrapping and immersed for a period of 20 minutes in a boiling solution having the same composition as the second, or stretching bath, to convert the yarn to regenerated cellulose. The yarn cake was removed from the regenerating bath, was washed free of occluded salts, was treated with a lubricating finish and was dried. The final yarn possessed a dry tenacity of 4.32 grams per denier, a wet tenacity of 3.49 grams per denier and a dry elongation of 5.9%.

#### Example II

A viscose solution containing 7% cellulose and 9% sodium hydroxide and ripened to a common salt (sodium chloride) index of 1.8 was extruded through a spinnerette, into a bath prepared from 15% borax, 15% sodium sulfate, 5% ammonium sulfate and 65% water, together with sufficient sulfuric acid to yield a pH of 4.1, the bath being maintained at a temperature of 60° C. After a bath travel of 6 inches at no substantial tension and an air travel of 8 inches, the yarn was passed onto the first of two stretching drums at a speed of 450 inches per minute. It was then led for a distance of 20 inches through a second bath prepared from 10% borax, 10% sodium sulfate and 80% water with sufficient sulfuric acid to yield a pH of 6.0 and maintained at a temperature of 100° C. The yarn was removed from this bath by means of the second stretching drum rotating at a peripheral speed of 1,550 inches per minute, the yarn having been stretched to a length of 3.44 times its original length (244% stretch) during its travel through the last bath. The yarn was further processed as described under Example I except a regenerating bath prepared from 20% sodium sulfate, 6% sulfuric acid and 74% water was used at 30° C. and for a period of 10 minutes. The final yarn possessed a dry tenacity of 5.02 grams per denier, a wet tenacity of 3.52 grams per denier and a dry elongation of 6.4%.

#### Example III

Viscose ripened to a common salt (sodium chloride) index of 3.4 and containing 8% cellulose and 9% sodium hydroxide was extruded through a spinnerette into an aqueous solution prepared from 17.4% borax, 17.2% sodium sulfate and 5.1% ammonium sulfate and 60.3% water and adjusted to a pH of 4.3 by the addition of suitable amount of sulfuric acid, the bath being maintained at a temperature of 70° C. The filaments passed through this bath a dis-

tance of 6 inches at no substantial tension, then through air for a distance of 8 inches, around a feed wheel at a linear speed of 900 inches per minute, and through a second bath for a distance of 20 inches, the second bath being formed from an aqueous solution containing 10% borax, 10% sodium sulfate and 80% water adjusted to a pH of 6.0 with sulfuric acid and maintained at a temperature of 100° C. The yarn was then passed around a second feed wheel driven at such a speed as to stretch the yarn about 185% during its passage through the second bath. The stretched yarn was collected in the manner described in Example I as unregenerated cellulose xanthate, was wrapped in a suitable cloth covering and was regenerated by being immersed for a period of 10 minutes in a bath consisting of 20% sodium sulfate, 6% sulfuric acid and 74% water maintained at 30° C. The regenerated yarn obtained was then passed in cake form under purifying and treating showers and finally dried. The final yarn possessed a dry tenacity of 4.08 grams per denier, a ratio of wet to dry tenacity of 0.85, and dry and wet elongations of 9.2% and 9.1%, respectively.

#### Example IV

A viscose solution ripened to a common salt (sodium chloride) index of 2.0 and containing 5.5% cellulose and 9% caustic was extruded into an aqueous bath containing 15% borax, 15% sodium sulfate, 5% ammonium sulfate and 65% water adjusted to a pH of 4.5 by suitable additions of sulfuric acid, and maintained at 60° C. After a bath travel of 6 inches at no substantial tension, the yarn was passed for a distance of 140 inches through air and around the first stretching roller and was stretched 113% through a stretching bath of the following composition: 10% borax, 15% sodium sulfate and 75% water and heated to a temperature of 100° C. The stretched yarn was collected in a relaxed state as in Example I and was regenerated by immersion for 30 minutes in a boiling bath made up of 30% ammonium sulfate, 10% sodium sulfate and sufficient sulfuric acid to yield a pH of 4.5. The stretched yarn after being purified and dried as described in Example I possessed a dry tenacity of 3.81 grams per denier, a wet tenacity of 2.01 grams per denier, and wet and dry elongations of 6.0% and 6.2%, respectively.

#### Example V

A viscose containing 5% cellulose and 9% sodium hydroxide was spun at a common salt (sodium chloride) index of 2.0 into a spinning bath containing approximately 18% borax, 9% sodium sulfate, 9% glucose and 62% water, adjusted to a pH of 4.0 and maintained at 57° C. After passing through 6 inches of this bath without the use of guides, the coagulated filaments were withdrawn at 300 inches per minute and advanced in a substantially tensionless condition through 8 inches air travel and for 130 inches around a positively driven roller. The thread was then subjected to high tension and stretched to 3.40 times its original length (240% stretch) while passing through a second bath containing approximately 10% borax and 10% sodium sulfate, adjusted to a pH of 5.6 and maintained at the boiling point. The yarn was drawn from the second bath by a second positively driven roller at 1020 inches per minute and collected relaxed on a slowly moving table so as to form a traversed package. The water-soluble xanthate yarn was regenerated in

a bath of the same composition as the stretching bath, washed, finished and dried as in Example I. The final yarn had the following physical properties:

Dry tenacity ..... 5.34 grams per denier  
 Wet tenacity ..... 4.16 grams per denier  
 Ratio of dry:wet  
 tenacity ..... .78  
 Dry elongation ..... 6.0%  
 Wet elongation ..... 6.7%  
 Filament cross-  
 section ..... smooth, uncrenulated, round

*Example VI*

A viscose containing 7.9% cellulose and 9.1% sodium hydroxide was spun at a common salt (sodium chloride) index of 3.7 into a spinning bath containing 17.2% borax, 17.0% sodium sulfate, 5.0% ammonium sulfate and 60.8% water, adjusted to a pH of 4.3 and maintained at 63° C. After passing through 6 inches of this bath without the use of guides, the coagulated filaments were withdrawn at 900 inches per minute and passed through 8 inches of air travel and then 130 inches around a positively driven roller. The yarn was then stretched 50% or to 1350 inches per minute while passing through a second bath containing 10% borax and 10% sodium sulfate, adjusted to a pH of 6.0 and maintained at the boiling point. The yarn was drawn from the second bath by a second positively driven roller at 1350 inches per minute and collected, relaxed on a slowly moving table. After regenerating, washing, finishing and drying as previously described the yarn had the following physical properties:

Dry tenacity ..... grams per denier ..... 2.16  
 Wet tenacity ..... do ..... 1.14  
 Dry elongation ..... per cent ..... 21.7  
 Wet elongation ..... do ..... 30.0

*Example VII*

A viscose solution containing 8.1% cellulose and 8.85% sodium hydroxide and ripened to a common salt index of 5.0 was extruded through a spinnerette into a bath prepared from 24.3% borax, 18.4% ammonium sulfate and 57.3% water and adjusted to a pH of 7.6, the bath being at a temperature of 65° C. After a bath travel of 6 inches at no substantial tension and an air travel of 8 inches, the yarn was passed to a drawoff roller at a speed of 900 inches per minute. It was then led for a distance of 20 inches through a second bath of 9% borax, 9% sodium sulfate and 82% water maintained at a pH of 6.2 and a temperature of 95° C. The yarn was removed from this bath by means of a second drum rotating at a peripheral speed of 2475 inches per minute, the yarn having been stretched to a length of 2.75 times its original length (175% stretch) during its travel through the last bath. The yarn was regenerated in a bath containing 20.0% sodium sulfate, 6.0% sulfuric acid, 74.0% water at room temperature and thereafter was washed, finished and dried. The finished yarn had a dry tenacity of 3.61 grams per denier, a wet tenacity of 2.30 grams per denier with dry and wet elongations of 7.2 and 7.6 respectively.

*Example VIII*

Yarn was spun in the manner shown in Example VI but the coagulated yarn after passing 3 passes around the initial or drawoff wheel at 900 inches per minute was allowed to fall directly

onto a traversed table forming a package. This package was wrapped in cloth and regenerated in a bath of 10% borax, 10% sodium sulfate, having a pH of 6.0 and temperature of 100° C.

5 The yarn was then washed, finished and dried and possessed the following physical properties.

Dry tenacity ..... grams per denier ..... 0.95

Wet tenacity ..... do ..... 0.56

10 Dry elongation ..... per cent ..... 121

Wet elongation ..... do ..... 155

This yarn may be treated with liquid ammonia in accordance with Woodell, U. S. 2,462,927 to increase the elongation to about 250%.

15 The utility of the invention is dependent to a large extent on the precipitation of coagulation of the viscose independently of regeneration. The baths utilized in the above examples under the conditions present exert a strong and rapid coagulating effect on viscose without at the same time causing any substantial degree of regeneration of the coagulated xanthate structure. The pH of the coagulating bath is maintained within the range of 3.0 to 9.0 and preferably within the 20 range of 4.0 to 6.0. The beneficial effect of the borate ions in the bath is lost if the pH is outside the range of about 3 to about 9.

The coagulating bath contains 5% or more of a borate calculated for convenience as borax (Na<sub>2</sub>B<sub>4</sub>O<sub>7</sub>.10H<sub>2</sub>O); i. e., although much of the borate may be present as boric acid, nevertheless in stating that the coagulating bath liquid contains 5% or more by weight of borate, this signifies a weight calculation on the convenient 30 assumption that all of the borate is present as borax. It is obvious that the borate radical may be present in other forms, for example in the form of acid borate, hypoborate, metaborate, perborate as well as the tetra- or pyroborate and 35 as combined with alkali metal or ammonia. Similarly the coagulating bath also contains 5% or more of sulfate preferably as the result of sodium sulfate additions but sulfates of other bases may be used and sulfuric acid additions to 40 adjust the pH also contribute. For convenience the sulfate is often calculated as sodium sulfate (Na<sub>2</sub>SO<sub>4</sub>).

In describing the specific composition of the 45 borate-sulfate baths utilized in the above examples, it is to be understood that although the baths can be made up from commercially available materials so as to have approximately the desired pH, for instance by using boric acid or sodium bisulfate, nevertheless it is usually advisable to add a certain amount of mineral acid, e. g. sulfuric acid or its acid salts so as to adjust the pH of the bath accurately to the desired value. In general any other acid or acidic material may be used to get the desired pH.

60 Although the coagulating bath can comprise, if desired, an aqueous solution containing only alkali metal salts of boric and sulfuric acids in an amount of from 5 to 20% of each and preferably acid necessary to yield the desired pH, the bath may also contain other salts of strong acids.

65 Thus, as indicated in Examples II, III, IV, VI and VII the bath may also contain a substantial amount of ammonium sulfate, one typical form of such bath which is preferred being an aqueous solution containing 15% borax, 15% sodium sulfate and 7% ammonium sulfate, the bath being adjusted to a pH of, for example, 4.0 to 7.6. The addition of ammonium sulfate along with sodium or other sulfates or in place thereof is indeed important. This ammonium sulfate addition to

the spinning bath makes possible very substantial increases in speed of spinning as for example 2, 3 or more times the maximum speed attainable in borax-sulfate baths free of ammonium sulfate. The addition of as little as 1 or 2% ammonium sulfate will noticeably improve the rate of spinning while 5% or 10% or more will generally yield optimum results both in speed and quality of yarn produced. Another material that can be added to the borate-sodium sulfate baths with advantage is glucose or other polyhydric alcohol such as glycerine or a glycol, as indicated in Example V.

The total salt concentration in the bath may range from 10% to 55% with amounts of 20% to 45% being preferred. Thus, a bath containing 40% ammonium sulfate and 15% borax may be used. Concentrations leading to salt crystallization on guide surfaces, etc., are generally avoided.

The coagulating bath is preferably maintained at a temperature of 45° to 75° C., the yarn travel through the bath preferably being of the order of 2 inches to 18 inches. However, these temperatures and bath travels are not critical, provided only that they are not so great as to cause any substantial degree of regeneration of the cellulose xanthate structures produced therein. Since spinning requires but a few seconds, very little regeneration occurs at the higher temperature. The yarn must, however, be preferably completely coagulated before it is subjected to the subsequent stretching operation of the invention. When, as in certain of the examples, the travel through the coagulating bath is insufficient to completely coagulate the extruded viscose, it is desirable to lag the incompletely coagulated yarn under low tension, for example, by passing it through air, for a time sufficient to complete the coagulation. Or, if desired, the yarn can be passed through a second borate-sulfate coagulating bath for a period of time sufficient to complete the coagulation. If the yarn is not completely coagulated prior to stretching, the amount of stretch obtainable will be distinctly impaired.

It is important, to obtain the full advantages of the invention, for coagulation to take place under conditions of very low tension. Thus, the tension imposed on the filaments in the coagulating bath should not be in excess of 0.1 gram per denier and preferably not in excess of 0.01 gram per denier. Where the viscose structure is non-filamentary, tensions equivalent to those given in connection with filaments will be used.

The stretching of the coagulated-only yarn obtained in the course of this invention can be accomplished by passing the yarn about positively driven pairs of stretching rolls or in any other known manner. In accordance with the examples, this stretching is preferably performed while the yarn is passing through a bath of the same general type as the coagulating bath, but heated almost to the boil since such baths assist in developing the greatest degree of stretch. However, this is not essential. The stretching operation can, if desired, be performed in the presence of an aqueous solution of inorganic salts, a liquid such as glycerin, triethanolamine, ethylene glycol, etc., or even in the presence of a gaseous medium such as live steam, air, carbon dioxide, sulfur dioxide, etc. These stretching media are preferably maintained at an elevated temperature, for example, 100° C. or more. However, this is not critical to the practice of the invention and they can, if desired, be maintained at any

other temperature, for example, at room temperature. In accordance with the principles of this invention, the yarn at the start of the stretching operation is substantially unregenerated and is water-soluble. The duration of the stretching operation and the contact of the yarn with the stretching medium is preferably so short that no substantial amount of regeneration is effected. This is not critical to the practice of the invention however and, if desired, the yarn may be partially or completely regenerated during the stretching operation.

The stretched yarn is then collected in suitable package form and regenerated. It may be collected on a rotating bobbin in the form of a cross-wound package or in a centrifugal bucket of the type customarily employed in the spinning of viscose rayon yarn, or it may be collected in any other package form. Preferably, however, the 15 yarn is permitted to fall in a relaxed, tensionless state on to a slowly moving support and formed into a cake-like package in the manner of Example I above. The yarn package protected by a suitable cover is then treated with a regenerating bath for a suitable period of time. This bath can comprise a mineral acid solution, for example of the type generally employed in the single bath process in the spinning of viscose rayon yarn and containing from 8% to 10% sulfuric acid, together with varying amounts of inorganic salts such as sodium sulfate, etc., or it may comprise an aqueous inorganic salt solution or an inert liquid (such as glycerin) heated to a high temperature. It may comprise a boiling 20 solution of the same general type as the coagulating or stretching baths of this invention. Preferably, however, the regenerating bath is an acid salt bath comprised of about 6% sulfuric acid and 20% sodium sulfate maintained at a temperature of about 30° C. On the other hand, the 25 yarn wet with occluded coagulating bath and stretching bath liquors can be regenerated by spontaneous decomposition of the cellulose xanthate by permitting it to stand a sufficiently long time (for example 24 hours) at room temperature. In such a case, of course, the humidity of the surrounding atmosphere should be maintained sufficiently high to prevent crystallization within the yarn of those salts contained in the occluded liquors.

It is not necessary that the yarn be regenerated and purified in package form. The coagulated-only yarn can be led through a regenerating bath in a continuous manner prior to its collection in package form, or the yarn can be collected in a relaxed, tensionless manner on a slowly moving conveyor belt of the type shown in British Patent No. 379,880 to Topham, the yarn, collected in the form of small overlapping ringlets, being subsequently led under showers of regenerating and purifying liquids and dried. The invention can be applied to continuous spinning, purification and collection processes of any character.

Although any method can be used in preparing the viscose utilized in the practice of the invention, the viscose employed in the examples was prepared by a standard method involving the combination of alkali (soda) cellulose with 26% carbon bisulfide based on the cellulose content of the alkali cellulose. Also, viscoses having a wide range of viscosities may be used, e. g. from 64 to 960 poises. Viscoses which have been submitted to a very short or very long ripening period may be used to good advantage as, for example, a high salt index viscose (4.0 or more) or a low salt

index viscose (2.0 or less). The use of the strong coagulating baths of this invention causes rapid coagulation of a high index viscose as well as low index viscose. It is also preferred, although not critical, that the alkali cellulose used be subjected only to a short aging period.

It is preferred, in order to develop the greatest stretchability of the coagulated, unregenerated structures, to utilize viscose in which the caustic content is higher than the cellulose content, e.g. a viscose containing 7% cellulose and 9% sodium hydroxide. However, other viscoses which have a sodium hydroxide content less than the cellulose may also be used and, generally speaking, viscoses having a cellulose or caustic content of between 4% and 9%, or more, are quite satisfactory.

From the above description, it is clear that the present invention makes possible the continuous rapid formation of thoroughly coagulated filaments which can be stretched so as permanently to increase their length 100%, 150%, 200% and more, this degree of extensibility being far beyond that possessed by cellulose xanthates produced according to previously known processes. Filaments and yarn formed by converting such coagulated structures to regenerated cellulose possess a ratio of wet to dry tenacity of 0.70 and higher, and possess a dry tenacity of 5.0 grams per denier and higher. The new yarns of this invention furthermore withstand severe treatments such as washing, treatment with swelling agents, etc. with little if any loss in strength.

Filaments spun in accordance with the preferred process of this invention furthermore possess a smooth, uncrenulated surface. Moreover, they resemble in their cross-sectional dimensions, the shape of the spinnerette orifices through which the viscose solution is extruded into the coagulating only bath. The size and number of holes in the spinnerettes used in the practice of the invention are not critical since any standard spinnerette, e.g. one containing 40 holes and generally of the type used in the production of 150 denier yarn according to ordinary rayon manufacturing methods is satisfactory. Such spinnerettes normally have a hole size of 0.003 inch, but it has been found, in the exercise of this invention, that a spinnerette hole size of less than 0.003 inch gives somewhat better results.

The improved coagulating baths provided by this invention not only make it possible to produce a yarn of very desirable properties, but also make possible a spinning process that is admirably adapted for use on a commercial scale. The process does not require the use of complicated apparatus or difficultly prepared baths. Moreover, the ingredients employed are relatively inexpensive.

The invention has its principal utility in the manufacture of filaments and yarns. However, the invention, broadly speaking, is applicable also to the production of thin tubing and other types of products by the viscose process with the attaining of generally the same advantages which result from the use of the invention in the manufacture of filaments and yarns.

We claim:

1. A process which comprises precipitating viscose in an aqueous bath having a pH of 3.0 to 9.0 and containing dissolved therein salts in such an amount as to rapidly coagulate the viscose without substantially regenerating the coagulated cellulose xanthate, a portion of said salts being a borate present in amounts equivalent to at least 5% borax.

2. A process in accordance with claim 1 in which a portion of said salts is a sulfate present in amounts equivalent to at least 5% sodium sulfate.

3. A process in accordance with claim 1 in which the total concentration of said salts is from 10% to 55%.

4. A process in accordance with claim 1 in which the total concentration of said salts is from 20% to 45%.

5. A process which comprises precipitating viscose in an aqueous bath having a pH of 3.0 to 9.0 and containing salts dissolved therein in such an amount as to rapidly coagulate the viscose without substantially regenerating the coagulated cellulose xanthate in the absence of substantial tension, a portion of said salt being a borate present in amounts equivalent to at least 5% borax.

6. A process which comprises precipitating viscose in an aqueous bath having a pH of 3.0 to 9.0 and containing dissolved therein salts in such an amount as to rapidly coagulate the viscose without substantially regenerating the coagulated cellulose xanthate and stretching the resultant product, a portion of said salt being a borate present in amounts equivalent to at least 5% borax.

7. A process which comprises precipitating viscose in an aqueous bath having a pH of 3.0 to 9.0 and containing dissolved therein salts in such an amount as to rapidly coagulate the viscose without substantially regenerating the coagulated cellulose xanthate, a portion of said salts being a borate present in amounts equivalent to at least 5% borax; and stretching the resultant product in the presence of an aqueous medium containing dissolved therein a substantial amount of borate.

8. A process which comprises precipitating viscose in an aqueous bath having a pH of 3.0 to 9.0 and containing dissolved therein a borate and a sulfate in such an amount as to rapidly coagulate the viscose without substantially regenerating the coagulated cellulose xanthate, stretching the resultant product and, after the stretching is completed, converting the stretched xanthate to regenerated cellulose.

9. A process which comprises precipitating viscose in an aqueous bath having a pH of 3.0 to 9.0 and containing dissolved therein a borate and a sulfate in such an amount as to rapidly coagulate the viscose without substantially regenerating the coagulated cellulose xanthate, stretching the resultant product, and then converting the stretched xanthate to regenerated cellulose while in the relaxed state.

10. A process of manufacturing regenerated cellulose yarn which comprises extruding viscose into a bath having a pH of between 3.0 and 9.0 and containing dissolved therein at least 5% each of a borate and a sulfate, calculated as borax and sodium sulfate, respectively, under very low tension conditions, stretching the resultant cellulose xanthate filaments at least 100%, and converting the stretched cellulose xanthate filaments to regenerated cellulose.

11. A process of manufacturing regenerated cellulose yarn which comprises extruding viscose into a bath having a pH of between 3.0 and 9.0 and containing dissolved therein at least 10% each of a borate and a sulfate, calculated as borax and sodium sulfate, respectively, under very low tension conditions, stretching the resultant cellulose xanthate filaments at least

## 11

150%, and converting the stretched cellulose xanthate filaments to regenerated cellulose while in the relaxed state.

12. A process of manufacturing filaments of regenerated cellulose which comprises extruding viscose under very low tension conditions into a bath having a pH of between 4.0 and 6.0 and containing dissolved therein at least 10% each of a borate and a sulfate calculated as borax and sodium sulfate, respectively, and not less than 5% ammonium sulfate, imparting a high degree of stretch to the resultant cellulose xanthate filaments and converting the stretched cellulose xanthate yarn to regenerated cellulose.

13. A coagulating bath for viscose comprised of at least 5% each of a borate and a sulfate calculated as borax and sodium sulfate, respectively, and maintained at a pH of from 3.0 to 9.0.

## 12

14. A coagulating bath in accordance with claim 13 heated to a temperature of 45° to 75° C.

15. A coagulating bath for viscose comprised of at least 10% each of a borate and a sulfate calculated as borax and sodium sulfate, respectively, and maintained at a pH of from 3.0 to 9.0.

16. A coagulating bath for viscose comprised of at least 10% borax, at least 10% sodium sulfate and at least 5% ammonium sulfate and maintained at a pH of from 3.0 to 9.0.

17. A coagulating bath for viscose comprised of at least 10% borax and at least 5% ammonium sulfate and maintained at a pH of from 3.0 to 9.0.

WESTON ANDREW HARE.  
FRANK KERR SIGNAIGO.

No references cited.